

(No Model.)

J. PARAVICINI.

ROLLER FOR PRINTING SOLID GROUND COLORS ON WALL PAPER  
AND METHOD OF MAKING SAME.

No. 513,822.

Patented Jan. 30, 1894.

Fig. 1.



Fig. 2.



Fig. 3.



WITNESSES:

H. L. Ourand.

J. L. Goombs

INVENTOR,  
Joseph Paravicini,  
J. Louis Berger &  
Attorneys

# UNITED STATES PATENT OFFICE.

JOSEPH PARAVICINI, OF BRISTOL, PENNSYLVANIA, ASSIGNOR TO CHARLES A. WILSON, OF SAME PLACE.

## ROLLER FOR PRINTING SOLID GROUND COLORS ON WALL-PAPER AND METHOD OF MAKING SAME.

SPECIFICATION forming part of Letters Patent No. 513,822, dated January 30, 1894.

Application filed September 15, 1893. Serial No. 485,589. (No model.)

*To all whom it may concern:*

Be it known that I, JOSEPH PARAVICINI, a citizen of the United States, and a resident of Bristol, in the county of Bucks and State 5 of Pennsylvania, have invented certain new and useful Improvements in Rollers for Printing Solid Ground Colors on Wall-Paper and Methods of Making the Same; and I do hereby declare that the following is a full, clear, and 10 exact description of the invention, which will enable others skilled in the art to which it appertains to make and use the same, reference being had to the accompanying drawings, which form a part of this specification.

15 My invention relates to improvements in rollers for printing solid ground colors on wall paper, and in the method of making the same. It is a great desideratum in rollers of this character to have the same absorbent, as 20 not only is the printing thereby rendered more perfect but there is a very large saving in the coloring material used. Attempts have heretofore been made to construct an absorbent roller for the above purpose by cementing a sheet of felt or other similar material to a rubber, iron or wooden roller. Such, however, is very defective in that the seam formed by the meeting or overlapping edges of the felt interfere with the proper working 25 of the roller and causes an inferior quality of work to be produced.

The object of my invention is to remedy the above and other defects and provide an absorbent seamless printing roller which will 30 perform its work in a very efficient and satisfactory manner.

The invention consists in the novel roller and the method of making the same, herein-after fully described and claimed.

40 In the accompanying drawings: Figure 1 represents an elevation of a printing roller constructed in accordance with my invention. Fig. 2 is a central longitudinal section of the same. Fig. 3 is a cross section on the 45 line  $x-x$  Fig. 2.

In carrying my invention into effect I take what is known as padding, (a cloth made from

the sweepings of cotton mills, and used in the manufacture of harness) and cut the same into circular washers of suitable diameter. 50 These washers are tied in bunches, and soaked in a hot solution of glue until thoroughly saturated. They are then taken and while yet in a hot state put upon a tube or shaft, and subjected to great pressure whereby a solid, homogeneous roller is produced. The roller thus formed is left in the press until dry when it is transferred to a lathe and turned to within a short distance of the required size. It is then dipped into a vat containing a solution 60 of glue, water and clay white, in which it is boiled until thoroughly saturated. It is then again dried, when it will become very hard and rough. It is now put in a lathe and turned to the required size, and is then subjected to a thorough rubbing with pumice stone and water. The water and stone wash out the hardening ingredients to a depth of about a quarter of an inch, leaving an absorbent face which will take and retain the 70 coloring matter used for printing, and a hard center or body.

In the said drawings the reference numeral 1 designates the tube or shaft and 2 the body of the roller constructed as above described. 75

The numeral 3 designates heads fitted onto the mandrel either after completion of the roller or while it is being made. They are preferably placed on the tube or shaft, just before the first turning operation takes place. 80 Between these heads and the ends of the rollers are placed brass washers 4.

Having thus described my invention, what I claim is—

1. The method herein described of making 85 rollers for printing solid ground color on wall paper, the same consisting in taking washers of fibrous or textile material, soaking them in a hot solution of glue, then placing them on a shaft or tube and subjecting them to pressure, then drying the same and turning in a lathe to near the required size, then dipping in a boiling solution of glue, water and clay white, then drying and turning in a lathe to 90

the required size, and finally rubbing with pumice stone and water; as and for the purpose specified.

2. As an improved article a printing roller consisting of a tube or shaft and a body of compressed fibrous or textile material having a hard solid center and an absorbent face or periphery; substantially as described.

In testimony that I claim the foregoing as my own I have hereunto affixed my signature to in presence of two witnesses.

JOSEPH PARAVICINI.

Witnesses:

WILLIAM C. ALLOWAYS,  
JOHN G. STREET.